

Nov. 8, 1932.

K. EMMEL

1,887,453

METHOD OF PRODUCING CAST IRON OF HIGH QUALITIES  
OF STRENGTH IN A CUPOLA FURNACE

Filed March 6, 1928



Inventor:  
Karl Emmel

By Watson, Coit, Morse + Grindle  
Attys

## UNITED STATES PATENT OFFICE

KARL EMMEL, OF MULHEIM-RUHR, GERMANY

## METHOD OF PRODUCING CAST-IRON OF HIGH QUALITIES OF STRENGTH IN A CUPOLA FURNACE

Application filed March 6, 1928, Serial No. 259,809, and in Germany March 15, 1927.

- Thorough experiments have proved that a smelting made according to the process for the production of iron castings with a low carbon content and of particularly high qualities, as described in the specification of my prior Patent No. 1,683,714, has the property of maintaining said high qualities of strength even if it is subjected to a subsequent carbonization.
- 10 The invention is based upon this fact, and its object is, as a further improvement or modification of the process afore-mentioned, to produce iron castings which beside their high qualities of strength have a particular favorable capability of being conveniently worked.
- The improved method forming the subject matter of the present invention consists in, first, producing, according to the process aforementioned, a superheated smelting of 20 a total carbon content of about 2-3% from a charge whereof the iron portion consists of at least 50% of iron low in carbon while the remainder of the iron contents consists of iron rich in carbon and of suitable admixtures and 25 wherein the quantity of coke employed amounts to between 9 and 13% of the total charge that is submitted to a varying blast pressure of between 400 and 800 mms. water gauge pressure, and, subsequently, carbonizing said smelting low in carbon to a higher carbon content, for instance 3.4-3.6%.
- Beside the favorable capability of working the product obtained, which does not in any way impair the high qualities of strength of 35 the same, the further advantage is attained that the subsequent carbonization reduces the solidification point of the smelting and favorably influence the casting capability of the latter.
- 40 The improved method can, according to the invention, for instance, also be carried out within the same cupola furnace, in which the melting of the charge was done, by the subsequent carbonization of the superheated 45 smelting low in carbon being produced in the lower part of the cupola furnace by the heating coke of the latter. The degree of carbonization can be controlled by a regulation of the carbonization time or of the height 50 of the bath in the receiver of the cupola fur-
- nace, or by a change of the height of the melting zone.
- In the accompanying drawing, one form of cupola furnace, in which the improved method may be satisfactorily practiced, is illustrated by way of example. The shell or wall of the furnace is indicated at 10, upper and lower tuyères at 11 and 12 respectively, and tapping holes at 13 and 14. The body of coke is shown to occupy the lower end of the smelting chamber, below the tuyères, and the charge of iron and carbon the bulk of the remainder of the space available. The relationships of the diameter of the combustion space to the distances of the tuyères from the bottom, respectively, are set forth, the lower set of tuyères being preferably located at a distance above the bottom equal to three fourths of the diameter of the combustion space, and the upper tuyères being one and one fourth diameters above the bottom. These dimensions are, of course, approximate.
- I am aware that it has already been proposed for instance in the U. S. Patent 1,336,256 (Muntz and Roubien) to work a 55 cupola furnace with a deep lower part in such a way that, first, the heating coke is brought to incandescence by an upwardly directed blast and, then, the casting scraps are molten, which smelting is to form at the rear 60 of the tap-hole at the bottom of the furnace a liquid cast-iron layer of slow solidification due to its less high carbon content. Only then, the remaining charge or burden consisting mainly of steel scraps is to melt 65 down. The result of said proposal would be—like in the last-mentioned mode of carrying out the improved method forming the subject matter of the present invention—a carbonization of the steel smelting in the 70 lower part of the furnace, which result has, however, been neither foreseen nor stated as a consequence of said proposal, for otherwise the precaution against solidification at the rear of the tap-hole is not understood. Fur- 75 thermore, said proposal of the Patent 1,336,256 did not aim at the superheating of the smelting or at the production of a smelting of particularly favorable casting capability. This is also contradicted by the 80

fear in said proposal of a solidification of the smelting already in the furnace itself. Said known proposal had for its only object to cheapen the charge principally designed for an adjoining Bessemer process, without the 5 perception of the high value, of the idea upon which the present invention is based, for the production of iron castings of high qualities of strength, and so on.

The present invention has for its object, 10 to produce in a simple cupola furnace such castings of specially high values, which possess besides high resistance values still specially favorable capability for treatment. It consists in utilizing the high superheating, 15 which in the cupola furnace is due to the steel containing smelting, to obtain a good distribution of the carbon at subsequent carbonization without the necessity to use, as hitherto, several devices for smelting and carbonizing, 20 only one single device and only one single smelting operation being required. This is obtained by arranging the device specially for the subsequent carbonizing by suitably spacing the tuyères from the bottom plate of 25 the furnace and by providing a suitable number of rows of tuyères and further by conducting the operation of the furnace in such a manner, that a very high temperature of the smelting is attained.

30 At an inner diameter of the furnace of 900 mm there has been obtained, for instance at a distance of 450 mm. of the tuyères from the bottom plate of the furnace, 2,8 to 3,1% of 35 carbon content of the cast iron. If however the first row of tuyères is spaced 600 mm from the furnace bottom, the cast iron shows a percentage of carbon from 3 to 3,4%. This shows that a subsequent carbonizing of the 40 superheated smelting, obtained by the smelting process with high steel charge, is the more possible the greater the distance of the nozzles from the furnace bottom is selected.

The layer of the hottest working of the 45 furnace is situated about 30 cms. above the tuyères and, if there are several rows of tuyères, higher plus the distance between the several rows of tuyères. There have been proposed therefore two means for the subsequent carbonizing, i. e. first the increasing 50 of the distance between the furnace bottom and the first row of tuyères and secondly increasing the height of the layer of the hottest furnace working above the 55 tuyères by arranging several rows of tuyères. The producing develops in such a manner that first in the specially thick layer of the hottest furnace working above the tuyères the steel charge is heated to the highest 60 possible temperature, and this excessively heated smelting is then subsequently thoroughly carbonized underneath the tuyères in the comparatively high layer of filling coke. This space in the furnace between the furnace 65 bottom and the tuyères is filled with coke in a

manner known per se. The molten iron takes up the carbon from this coke.

According to the smelting process of the invention, the object of placing the layer of the hottest furnace working at a higher lever 70 is, to obtain the highest possible superheating in order to subsequently carbonize thoroughly this highly heated smelting with the aid of a high layer of filling coke. From the high superheating of the smelting results a 75 quite specially fine distribution of the carbon in the smelting so that a product can be obtained, which is equal to the best cast iron-products known at present.

The improved method can, for instance, 80 be put into practice in such a way that the smelting of low carbon content attained above the tuyères and heated to steel melting temperature is passed through and carbonized in the coke-filled smelting receiver prior to its 85 admission to the forehearth. Also in this case the degree of carbonization of the smelting can be controlled by a regulation of the bath in the smelting receiver. With a long stay 90 of the smelting in the lower part of the furnace serving as a carbonization chamber, or with a slow passage of the smelting therethrough, the latter will receive a higher carbon content than with a shorter stay and with 95 a larger velocity.

The height of the carbonizing smelting receiver, or the height of the bath respectively, can be regulated with a maintenance of the height of the tuyères, by filling-in the bottom end of the lower part of the furnace 100 with suitable substances, such as sand, fire-bricks, or the like, for making the bottom of the furnace of different heights.

The subsequent carbonization of the smelting low in carbon and thus taking indeed advantage of the maximum temperatures in the furnace, can also take place substantially or in addition to the afore-mentioned provisions by performing the melting process of the charged low-carbon iron, for a comparatively 110 high layer of highest temperature, above as well as within the uppermost partial layer thereof, and that in such a way for the smelting produced has occasion to be heated to, or at least approximately to said highest temperature in the furnace. Additionally thereto, the superheated smelting low in carbon thus formed has then in the lower partial layers 115 of the artificially created particularly high layer of highest furnace temperature occasion to become carbonized, and that just at said high smelting superheating temperature. As a means for influencing the height of said layer of hottest furnace working, it is proposed to arrange the blast tuyères in several 120 superposed rows in a way known in the art for different purposes to mine.

The above statements show to anyone versed in the art the way how, on the one hand, by a systematic utilization of the ef- 130

fects of such a zone of hottest furnace working a controllable subsequent carbonization of a superheated smelting low in carbon can be obtained, and how, on the other hand, the 5 final carbon content of the product leaving the furnace can be directly influenced by a regulation of height of said layer or zone of hottest furnace working.

It may be noted that a regulation of the 10 height of such a layer or zone of hottest furnace working can also be attained with the aid of one single row of tuyères, by changing the quantity of blast supplied per unit of time, if required, with a simultaneous 15 charge of the pressure of the blast. Then, by an increased supply of blast with a maintenance of the usual quantities of coke, an heightening of said layer or zone can be obtained with the stated action upon 20 an increase of the carbon content of the smelting finally produced.

Thorough experiments have unobjectionably proved the effective applicability of the new rules upon which the improved method 25 is based. The details of the latter depend, of course, upon the dimensions and the construction of the cupola furnace used and can be easily determined for each individual case by a series of trials.

30 What I claim, is:

1. The method of operating a cupola furnace in the production of cast iron which consists in introducing into the furnace chamber a charge of iron and coke, at least 25 50% of the iron so introduced being in the form of steel or wrought iron of low carbon content and the coke comprising not more than about 13% of the total charge, submitting the charge, after ignition of the coke, to 40 the action of an air blast under water gauge pressure of between 400 and 800 mm. to effect smelting of the metallic charge, whereby a molten metal of relatively low carbon content but extremely high temperature is 45 produced, and thereafter passing this superheated metal through a body of coke to increase the carbon content thereof.

2. The method set forth in claim 1 which includes the step of regulating the degree of 50 carbonization below the tuyères by varying the height of the tuyères above the furnace bottom.

In testimony whereof I have hereunto set my hand: